

## UNITED STATES PATENT OFFICE

2,097,609

## CONCENTRATION OF GOLD BEARING MATERIALS

Stanley Tucker, London, England, assignor to Minerals Separation North American Corporation, New York, N. Y., a corporation of Maryland

No Drawing. Original application January 24, 1935, Serial No. 3,267. Divided and this application May 22, 1937, Serial No. 144,314. In Great Britain January 30, 1934

9 Claims. (Cl. 209—166)

This application is a division of my co-pending application Serial No. 3267, filed January 24, 1935.

The present invention relates to an improved process of extracting gold from ores and like materials by a form of physical concentration depending upon the surface properties of the material under treatment, such for example as froth flotation, and has for its general object 10 to provide for simplicity in such extraction, as well as for high gold recovery and high gold assay of concentrate.

In accordance with the invention, the gold-bearing material in the state of finely-divided 15 particles is formed into a pulp with water both in the presence of a mercurial agent and in the presence of an organic sulphur derivative of carbonic acid. By this combination of substances, as discovered, the gold particles present in the pulp are so modified at their surfaces 20 that they are made amenable to subsequent concentration depending upon their surface properties.

Instead of the organic sulphur derivative of 25 carbonic acid, a sulphidizing agent has also been found capable of use along with the mercurial agent to produce the stated effect on the gold particles present in the pulp, the use of sulphidizing agents in this manner being separately 30 claimed in the aforementioned application Serial No. 3,267.

In applying the process in apparatus of the kind ordinarily employed for froth flotation and in conjunction with usual frothing agents so 35 that the concentrate floats in the form of a froth, it has been found that under suitable conditions an almost complete recovery of gold can be obtained by the process in the form of a high grade concentrate.

The surface-modifying agents may be dispersed 40 among the particles of the gold-bearing material during an agitation or grinding operation, carried out prior to concentration.

The mercurial agent may be metallic mercury 45 or a solution of a salt thereof. Mercuric chloride may be used dissolved in an excess of sodium cyanide, a slight excess being sufficient for the purpose. This solution is believed to result in the formation of a sodium mercuric cyanide, with 50 some free sodium cyanide present.

Alkali xanthates are of course included among 55 the organic sulphur derivatives of carbonic acid which may be employed in the process. As to the sulphidizing agents which have been found useful, they include sulphur, soluble sulphides or

polysulphides, and sulphur dissolved in sulphides or polysulphides.

Various other agents may be present when the surface-modifying agents are acting upon the gold particles, as during the above-stated preliminary agitation or grinding operation. The use in this manner of a tin salt, such as stannous chloride ( $SnCl_2$ ), has been found to reduce the quantity of the mercurial agent which is required.

The following is a description of a test which was made in carrying the invention into effect:

A 500 gramme sample of ore from Klerksdorp, South Africa, a partly oxidized gold ore containing iron sulphide, was comminuted so as to pass a screen having 10 meshes to the lineal inch and thereafter made into a pulp with 250 cubic centimeters of water. To this pulp mercury in the metallic state was added at the rate of 1.6 lbs. per ton, whereupon the pulp was ground in a pebble mill for forty minutes. After thirty minutes of this grinding, there were added to the mill 2 lbs. per ton of potassium xanthate, 0.45 lb. per ton of Anglo Persian fuel oil, 0.08 lb. per ton of pine oil, and 0.078 lb. per ton of blast furnace creosote. These additional agents were therefore ground with the ore for ten minutes.

The resulting material was about such as would pass a screen having 100 meshes to the lineal inch. It was subjected to froth flotation in a sub-aeration machine with two additions of 0.25 lb. per ton of potassium xanthate. As a result 30 97.7% of the gold in the ore was obtained in a concentrate which assayed 177.2 dwts. per ton, the original sample of ore assaying 12.29 dwts. per ton.

I claim:—

1. A process for the concentration of a gold-bearing material consisting in forming a pulp of finely-divided particles of the gold-bearing material with water in the presence of a mercurial agent and an organic sulphur derivative of carbonic acid, so that the surfaces of the gold particles in the pulp are modified by said mercurial agent and organic sulphur derivative of carbonic acid and said gold particles made amenable to concentration depending upon their surface properties, and concentrating said gold particles from the material by flotation.

2. A process for the concentration of a gold-bearing material consisting in forming a pulp of finely-divided particles of the gold-bearing material with water in the presence of a mercurial agent and an organic sulphur derivative of carbonic acid, so that the surfaces of the gold particles in the pulp are modified by said mercurial 50 agent.

- agent and organic sulphur derivative of carbonic acid and said gold particles made amenable to concentration depending upon their surface properties, and concentrating said gold particles from the material by froth flotation.
3. A process for the concentration of a gold-bearing material consisting in the preliminary step of agitating a pulp with water of finely-divided particles of the gold-bearing material in the presence of a mercurial agent and an organic sulphur derivative of carbonic acid, so that the surfaces of the gold particles in the pulp are modified by said mercurial agent and organic sulphur derivative of carbonic acid and said gold particles made amenable to concentration depending upon their surface properties, and the subsequent step of concentrating said gold particles from the material by flotation.
4. A process for the concentration of a gold-bearing material consisting in the preliminary step of grinding the gold-bearing material with water into a pulp of finely-divided particles in the presence of a mercurial agent and an organic sulphur derivative of carbonic acid, so that the surfaces of the gold particles in the pulp are modified by said mercurial agent and organic sulphur derivative of carbonic acid and said gold particles made amenable to concentration depending upon their surface properties, and the subsequent step of concentrating said gold particles from the material by flotation.
5. A process for the concentration of a gold-bearing material consisting in forming a pulp of finely-divided particles of the gold-bearing material with water in the presence of metallic mercury and an organic sulphur derivative of carbonic acid, so that the surfaces of the gold particles in the pulp are modified by said mercury and organic sulphur derivative of carbonic acid and said gold particles made amenable to concentration depending upon their surface properties, and concentrating said gold particles from the material by flotation.
6. A process for the concentration of a gold-bearing material consisting in forming a pulp of finely-divided particles of the gold-bearing material with water in the presence of mercuric chloride and an organic sulphur derivative of carbonic acid, so that the surfaces of the gold particles in the pulp are modified by said mercuric chloride and organic sulphur derivative of carbonic acid and said gold particles made amenable to concentration depending upon their surface properties, and concentrating said gold particles from the material by flotation.
7. A process for the concentration of a gold-bearing material consisting in forming a pulp of finely-divided particles of the gold-bearing material with water in the presence of a mercurial agent and an organic sulphur derivative of carbonic acid, so that the surfaces of the gold particles in the pulp are modified by said mercurial agent and organic sulphur derivative of carbonic acid and said gold particles made amenable to concentration depending upon their surface properties, said mercurial agent comprising mercuric chloride dissolved in an excess of sodium cyanide, and concentrating said gold particles from the material by flotation.
8. A process for the concentration of a gold-bearing material consisting in forming a pulp of finely-divided particles of the gold-bearing material with water in the presence of a mercurial agent and an alkali xanthate, so that the surfaces of the gold particles in the pulp are modified by said mercurial agent and alkali xanthate and said gold particles made amenable to concentration depending upon their surface properties, and concentrating said gold particles from the material by flotation.
9. A process for the concentration of a gold-bearing material consisting in forming a pulp of finely-divided particles of the gold-bearing material with water in the presence of a mercurial agent and an organic sulphur derivative of carbonic acid, so that the surfaces of the gold particles in the pulp are modified by said mercurial agent and organic sulphur derivative of carbonic acid and said gold particles made amenable to concentration depending upon their surface properties, said pulp being also formed in the presence of stannous chloride, and concentrating said gold particles from the material by flotation.

STANLEY TUCKER.